

March 20, 1956

H. E. RICKS

2,739,107

APPLYING PROTECTIVE METAL COATINGS ON REFRACTORY METALS

Filed July 26, 1952

Fig.1.



Fig.2.



WITNESSES:

*Ed. A. Melleskey*  
*Leon J. Faya*

INVENTOR

*Herbert E. Ricks.*  
BY  
*Frederick Shope*  
ATTORNEY

1

2,739,107

APPLYING PROTECTIVE METAL COATINGS ON  
REFRACTORY METALS

Herbert E. Ricks, Pittsburgh, Pa., assignor to Westinghouse Electric Corporation, East Pittsburgh, Pa., a corporation of Pennsylvania

Application July 26, 1952, Serial No. 301,016

6 Claims. (Cl. 204—37)

This invention relates to members of molybdenum metal and other similarly readily oxidized refractory metals with imperforate protective metal coatings applied to the surfaces of the members.

The refractory metals molybdenum, titanium and zirconium, are readily oxidized when exposed to an oxygen-bearing atmosphere at elevated temperatures. Thus, while molybdenum metal melts at 2625° C. in a non-oxidizing atmosphere, if the molybdenum metal is heated to 500° C. and higher in contact with air, oxygen or other oxidizing gas, it forms a readily volatile oxide such that when in contact with air at 700° C., the molybdenum metal gives off dense dark clouds of smoke consisting of molybdenum oxides and in a short while it is consumed.

It has been proposed to coat the surface of molybdenum metal with a protective layer of chromium or other oxygen-resistant metal which would prevent access of oxygen or other oxidizing vapor to the molybdenum and in this way enable the use of molybdenum metal at temperatures above 500° C. It is absolutely necessary that such applied protective layers be imperforate in order to be of any value. However, it has been impossible hitherto to provide an imperforate coating that would so exclude oxygen. For example, electrodeposits of chromium have been plated on members of molybdenum and such coatings appeared to be sound and without pores. However, on heating such chromium plated members to 600° C. to 700° C., microscopic cracks and previously unnoted pinholes admitted oxygen to the molybdenum metal so that a stream of molybdenum oxide smoke issued from each of these openings and in only a short time substantial volumes of the molybdenum metal adjacent to each such opening had disappeared because it had oxidized and the resulting volatile oxide had escaped.

In the art, extensive tests have been performed by highly skilled metallurgists and electroplaters in attempts to provide impervious and imperforate protective coatings of electroplated metal on molybdenum, all without any consistent success. Further, in many cases, the electroplated metal did not adhere properly to the molybdenum and on heating blisters were formed with resulting failure.

For making members for high temperature applications as in gas turbines, jet engines and other highly heated applications demanding great strength, molybdenum metal members would be satisfactory if they were protected by a well-bonded adherent coating of a metal resistant to oxygen at the elevated temperatures encountered in such service.

The object of the present invention is to provide members comprising a body of molybdenum, titanium or zirconium, with the entire surface of the body coated with a highly adherent, imperforate deposit of nickel phosphide, the applied deposit being partially diffused into the surface of the body.

A further object of the invention is to provide for applying to molybdenum, titanium, and zirconium metal bodies an imperforate surface coating of nickel phosphide

2

and heat treating the body with the applied coating to produce a well-bonded, imperforate coating over the entire surface of the body.

Other objects of the invention will in part be obvious and will in part appear hereinafter. For a better understanding of the nature and objects of the invention, reference should be had to the following detailed description and drawing, in which:

Figure 1 is a cross section through a member comprising a body of molybdenum with a bonded coating of nickel phosphide over the surface thereof; and

Fig. 2 is a cross section through a molybdenum member having applied to its entire outer surface a nickel phosphide layer and a superimposed electrodeposit of at least one of the group consisting of nickel, cobalt and chromium.

I have discovered a method for producing on members of molybdenum, titanium or zirconium metal an imperforate, highly protective surface coating of the order of 0.001 inch thickness, which coating is so well bonded and adherent to the metal that it will withstand elevated temperatures and will protect the metal from oxidizing atmospheres at such elevated temperatures for prolonged periods of time. Briefly, the method comprises plating on cleaned molybdenum metal a coating of nickel phosphide, cobalt phosphide or both over the entire surface of the member to a thickness of the order of 0.001 inch and then heat treating the member with the applied nickel phosphide coating to a temperature of about 600° C. to 1100° C. in an inert and non-oxidizing atmosphere to melt the nickel phosphide coating. It appears that during this heat treatment the applied nickel phosphide becomes imperforate, and a partial diffusion of the nickel phosphide coating into the molybdenum metal occurs to produce a highly adherent bonding therewith. The resulting imperforate coating is so well bonded to the refractory metal that it will not crack open or part therefrom under extreme conditions of service. Furthermore, the heat-treated nickel phosphide coating may be readily overplated with one or more electrodeposits of any of the metals of the group consisting of nickel, cobalt and chromium.

The invention will be detailed hereinafter specifically by reference to molybdenum metal but it will be understood similar procedures may be applied to titanium and zirconium metal. The invention may be applied not only to pure molybdenum, titanium and zirconium metal, respectively, but to alloys in which molybdenum, titanium and zirconium constitute at least 50% by weight. Thus, the invention may be applied to members comprising 95% molybdenum and 5% tungsten. Titanium may be modified with small amounts of chromium. Alloys of titanium containing a few per cent of chromium and up to 8% molybdenum, for example, may be treated in accordance with the present invention. It will be understood that zirconium ordinarily may contain a substantial amount of hafnium. Alloys containing mixtures of any two or all three of the metals molybdenum, titanium and zirconium with small amounts of various additional elements may be treated in accordance with the present invention. It will be understood that these alloys may contain small amounts of impurities which will not be detrimental to the application for the alloy.

## Example 1

Members of molybdenum metal are cleaned by first mechanically brushing, grinding and otherwise treating the surface to remove any impurities and blemishes thereon. The clean molybdenum member is then immersed in the following electrolyte:

|                  | Ounces per gallon |
|------------------|-------------------|
| Nickel sulphate  | 30                |
| Nickel chloride  | 7                 |
| Boric acid       | 4                 |
| Nickel phosphite | 5                 |

The pH of the electrolyte is 0.7. The electrolyte is at a temperature of 75° C. during plating. Plating current is passed through the molybdenum metal at a current density of 35 a. s. f. for one hour. This deposits over the entire surface of the molybdenum member a coating comprising over 85% nickel and the balance being phosphorus, the thickness being about 0.001 inch. The plated molybdenum member is then placed in a furnace provided with a hydrogen atmosphere and is heated slowly to a temperature of 550° C. over a period of time of four hours. The furnace temperature is then raised in 30 minutes to 800° C. The molybdenum member is maintained in the cooling chamber portion of the furnace where it does not reach a temperature much above 800° C., and thereafter the furnace temperature is increased to 1000° C. The plated molybdenum metal is then moved from the cooling chamber into the portion of the furnace at 1000° C. and kept there for 10 minutes. The molybdenum metal is then withdrawn and cooled to room temperature.

Members prepared as in Example I may be subjected to creep testing at 1800° F. at a loading of 20,000 p. s. i. At the end of many hours, the coating will be found to be completely impervious and will have perfectly protected the molybdenum metal from oxidation. The applied nickel phosphide coating will be oxidized only slightly.

The nickel phosphide coating will melt when heat treated and any excess above approximately 0.001 inch thickness will run off the member. After complete heat treatment, it has been found that the nickel phosphide comprises from 90 to 99% nickel with the balance being phosphorus. The average thickness of the heat-treated nickel phosphide coatings is approximately 0.0007 inch when it was originally plated to at least this thickness. If the plated thickness is less than 0.0007 inch, then the heat-treated nickel phosphide coating is the same thickness. The melting of the nickel phosphide deposit is necessary to produce an imperforate coating consistently.

Referring to Fig. 1 of the drawing, there is illustrated a cross section of a member produced in accordance with the process of this example. The body 10 of molybdenum metal has applied to all of its surfaces an exterior coating 12 of the heat-treated nickel phosphide deposit of a thickness of the order of 0.001 inch. The junction 14 between the nickel phosphide deposit 12 and the body 10 shows a slight diffusion and is characterized by no blisters, breaks or other perforations or faults.

The above aqueous electroplating electrolyte may be varied to provide from 25 to 35 ounces per gallon of nickel sulphate, from 6 to 9 ounces per gallon of nickel chloride hexahydrate, from 3 to 5 ounces per gallon of boric acid and from 4 to 6 ounces per gallon of the nickel phosphite. Good results have been secured in plating at current densities from 5 to 50 a. s. f. The pH of the electrolytes may vary from about 0.5 to 2 while the temperature of the electrolyte may vary from about 65° C. to 85° C.

The heat treatment of the applied nickel phosphide should be carried out in a non-oxidizing atmosphere such as cracked ammonia, hydrogen, helium, or argon for molybdenum metal members. Titanium and zirconium must be heat treated in a totally inert atmosphere comprising a noble gas, such as helium, argon or the like. In some cases, it may be desirable to heat treat the plated members in a vacuum, thereby eliminating any chance of contamination or causing undesirable results because of slight impurities in the heat-treating gas atmosphere surrounding the members.

In one test, nickel phosphide was placed in an evacuated furnace chamber and on raising the temperature

above 1200° C., the nickel phosphide vapors coated surfaces of members in the furnace. Titanium and zirconium members may be readily coated with nickel phosphide in such a vacuum furnace, the nickel phosphide being heated while the titanium or zirconium members are much cooler.

In order to provide better surface protection for resisting mechanical forces and wear and tear, the heat-treated nickel phosphide deposit is over-plated with one or more layers of at least one metal consisting of the group nickel, cobalt and chromium. Thus, a deposit of 0.002 inch of nickel or cobalt or alloys thereof may be plated over the nickel phosphide coating and then a substantial layer of chromium may be superimposed thereon. The following examples illustrate this feature.

#### Example II

A rod of molybdenum one-fourth inch in diameter was plated in the electrolyte of Example I to produce thereon a nickel phosphide layer of a thickness of 0.001 inch. The plated rod was then placed in a furnace provided with a cracked ammonia atmosphere and heated in accordance with the schedule set forth under Example I. The heat-treated rod was then placed in a nickel electrolyte having 40 ounces per gallon of nickel sulphate heptahydrate, 6 ounces per gallon nickel chloride hexahydrate, and 5 ounces per gallon of boric acid and plated at a current density of 40 amperes per square foot until a layer of nickel of a thickness of 0.002 inch was deposited thereon. The rod was then placed in a creep tester at 1800° F. under a load of 20,000 p. s. i. After passing 40 hours of this test, the rod was examined and was found to be in perfect condition and completely protected by the surface coating. Photomicrographs of cross sections through the rod showed a perfect bond between the nickel phosphide coating and the molybdenum metal. A slight oxidation was observed at the surface of the nickel coating due to its exposure to the air at 1800° F. for the test.

#### Example III

A rod was prepared by plating thereon 0.001 inch of nickel phosphide, heat treated as in Example I, and 0.002 inch thickness of nickel was plated thereon as in Example II; and the rod was further plated in a chromic acid plating electrolyte comprising 53 ounces per gallon of chromic acid and 0.53 ounce per gallon of sulphate, to deposit a 0.0015 inch thickness of chromium over the nickel layer. The rod was then placed in a creep tester where it was loaded at 20,000 p. s. i. at a temperature of 1800° F. After 100 hours under the test without failure, the rod was examined and found to be free from any oxidation of the underlying molybdenum metal. From all indications, the rod could have withstood this load at these temperatures for a much longer period of time.

Referring to Fig. 2 of the drawing, there is illustrated a cross section through a member produced in accordance with this Example III. A body 10 of molybdenum has plated thereon the nickel phosphide layer 12, then superposed thereon is a layer comprising electroplated nickel 16 and finally an exterior layer 18 comprising the electro-deposited chromium.

The nickel phosphide layer may be plated to a thickness of from 0.0001 to 0.002 inch; the deposits thinner than about 0.0007 inch preferably being protected by a superimposed coating of nickel, cobalt or chromium. During the heat treatment of the applied nickel phosphide coating, the coating melts and becomes imperforate, and partly diffuses and forms a highly adherent bond to the molybdenum metal surface. The melting point depends on the amount of phosphorus in the metal phosphide. Also, during heat treatment, a substantial part of the phosphorus leaves the coating, mostly by volatilization.

Cobalt sulphate, cobalt chloride and cobalt phosphite may be substituted in whole or in part for the nickel sul-

phate, nickel chloride, and nickel phosphite, respectively, in Examples I to III, thereby producing a composite cobalt-nickel phosphide deposit or an entirely cobalt phosphide deposit. These cobalt-containing phosphide deposits are otherwise treated identically as set forth herein.

While the electroplating process disclosed herein has given excellent results, it is feasible to produce a similar nickel phosphide coating by an immersion process wherein the molybdenum metal is immersed in an electrolyte of the type described in the November 1947 issue of the Journal of Research of the National Bureau of Standards in an article entitled "Deposition of nickel and cobalt by chemical reduction." Briefly, one such immersion solution comprises 30 grams of nickel chloride hexahydrate, 50 grams of ammonium chloride and 100 grams of sodium citrate per liter of solution, the balance being water. There is then added sufficient ammonium hydroxide to render the solution alkaline to a pH of from 8 to 10. When immersion plating is to be accomplished therein, the solution is heated to a temperature of from 190 to 200° F. and then 10 grams of sodium hypophosphite is added to each liter of solution. For every hour that plating is carried out in the solution, sodium hypophosphite is added to the bath at the rate of 5 grams per liter. This plating bath will build up a coating at the rate of 0.0003 inch per hour. Therefore, in an immersion period of from two to three hours, a sufficient thickness of nickel phosphide will be produced on the molybdenum metal. The resulting deposit is heat treated similarly to the nickel phosphide deposit described in the previous examples. It will be appreciated that cobalt salts may be substituted in whole or in part for the nickel salts in this immersion bath.

Since certain obvious changes may be made in the above procedures and different embodiments of the invention may be made without departing from the scope thereof, it is intended that all matter contained in the above description and drawing shall be interpreted as illustrative and not in a limiting sense.

I claim as my invention:

1. A member comprising a body of molybdenum metal and an imperforate coating of a thickness of the order of 0.001 inch applied to the entire surface of the body of molybdenum metal, the coating comprising essentially over 85% by weight of at least one metal selected from the group consisting of cobalt and nickel, and the balance being phosphorus, the applied coating being melted at from 600° C. to 1100° C. and partly diffused into the surface of the molybdenum.

2. A member comprising a body composed of at least 50% by weight of molybdenum metal and an imperforate coating of a thickness of substantially more than 0.001 inch comprising at least two layers applied to the entire surface of the body of molybdenum metal, the innermost layer of the applied coating being approximately 0.001 inch in thickness and comprising essentially over 85% by weight of at least one metal selected from the group consisting of nickel and cobalt, and the balance being phosphorus, the applied innermost layer being melted at from 600° C. to 1100° C. and partially diffused into the molybdenum, and superimposed on the innermost layer an adherent electrodeposit of at least one metal of the group consisting of nickel, cobalt and chromium.

3. A member comprising a body of a metal selected from at least one of the group consisting of molybdenum,

titanium, zirconium and alloys comprising at least 50% by weight thereof, an imperforate metal phosphide coating over the entire surface of the body of the metal, the coating comprising essentially at least 90% by weight of at least one metal selected from the group consisting of nickel and cobalt and the balance being phosphorus, the coating being of a thickness of the order of 0.001 inch and having been melted by heat treatment at a temperature of from 600° C. to 1100° C. after being applied to the body in order to diffuse it into the body of metal.

4. A member comprising a body of a metal selected from at least one of the group consisting of molybdenum, titanium, zirconium and alloys comprising at least 50% by weight thereof, an imperforate metal phosphide coating over the entire surface of the body of the metal, the coating comprising essentially from 90% to 99% by weight of at least one metal selected from the group consisting of nickel and cobalt and the balance being phosphorus, the coating being of a thickness of the order of 0.001 inch and having been melted by heat treatment at a temperature of from 600° C. to 1100° C. after being applied to the body, and an electrodeposit superimposed on the metal phosphide coating, the electrodeposit comprising at least one metal selected from the group consisting of nickel, cobalt and chromium.

5. In the process of producing imperforate protective coatings on a body of a metal selected from at least one of the group consisting of molybdenum, titanium and zirconium and alloys comprising at least 50% by weight thereof, the steps comprising electroplating on the entire surface of the body of the metal a thickness of the order of 0.001 inch of a metal phosphide composed of at least 85% metal and the balance being phosphorus from an electrolyte containing the chloride and from about 4 to 6 ounces per gallon of phosphite of at least one metal from the group consisting of nickel and cobalt, and heat treating the body of the electroplated metal phosphide coating at a temperature of from 600° C. to 1100° C. in a non-oxidizing, inert atmosphere to melt the electroplated coating so as to render it imperforate and to diffuse it into the body of the metal, the melted coating composed of from 90% to 99% by weight of the metal and the balance being phosphorus.

6. In the process of producing imperforate protective coatings on a body of a metal selected from at least one of the group consisting of molybdenum, titanium and zirconium and alloys comprising at least 50% by weight thereof, the steps comprising electroplating on the entire surface of the body of the metal a thickness of the order of 0.001 inch of a metal phosphide from an electrolyte containing the chloride and from about 4 to 6 ounces per gallon of a phosphite of at least one metal from the group consisting of nickel and cobalt, heat treating the applied metal phosphide coating at a temperature of from 600° C. to 1100° C. in a non-oxidizing atmosphere to melt it, and thereafter plating at least one metal from the group consisting of nickel, cobalt and chromium over the heat-treated metal phosphide coating.

#### References Cited in the file of this patent

#### UNITED STATES PATENTS

|           |                |               |
|-----------|----------------|---------------|
| 2,069,566 | Tuttle         | Feb. 2, 1937  |
| 2,594,933 | Knapp et al.   | Apr. 29, 1952 |
| 2,643,221 | Brenner et al. | June 23, 1953 |